

# UNITED STATES PATENT OFFICE.

HENRY LAVERS, OF CAMBERWELL, HENRY HOWARD GREENWAY, OF MELBOURNE, AND ALFRED HENRY PIPER LOWRY, OF PRAHRAN, VICTORIA, AUSTRALIA, ASSIGNEES TO MINERALS SEPARATION AMERICAN SYNDICATE (1913) LIMITED, OF LONDON, ENGLAND.

## CONCENTRATION OF ORES.

1,208,334.

Specification of Letters Patent. Patented Dec. 12, 1916.

No Drawing. Original application filed March 14, 1914, Serial No. 824,765. Divided and this application filed September 14, 1916. Serial No. 120,057.

To all whom it may concern:

Be it known that we, HENRY LAVERS, HENRY HOWARD GREENWAY, and ALFRED HENRY PIPER LOWRY, subjects of the King 5 of Great Britain and Ireland, and respectively residing at Camberwell, Melbourne, and Prahran, all in the State of Victoria, Commonwealth of Australia, have invented certain new and useful Improvements in 10 Concentration of Ores, of which the following is a specification.

This invention relates to improvements in the concentration of ores by flotation, and this application is a division of our application 15 filed March 14, 1914, Serial Number 824,765.

In this specification the term "ores" is intended to include concentrates, tailings, slimes and other products containing metalliferous mineral.

This invention relates to the concentration of ores by the agitation froth process, in which a froth of metalliferous mineral is floated to the surface of an ore pulp consequent upon the aeration and agitation of the pulp.

Hitherto froth flotation-separation has been conducted with the employment of an oily frothing agent such as is described in 30 Patent No. 835,120 of November 6, 1906, to Sulman, Picard and Ballot and in Patent No. 1,064,723 of June 17, 1913, to Greenway and Lavers, or with a soluble frothing agent such as is described in Patent No. 962,678 35 of June 28, 1910, to Sulman, Greenway and Higgins, the frothing agents disclosed in the last mentioned patent being of an organic nature and largely acid in character. A mineral acid such as sulfuric acid has been 40 used in addition to the frothing agent, acting in some manner not clearly understood to modify the qualities of the liquid and to assist the flotation of the metalliferous mineral and to retard or prevent flotation of 45 the gangue. In some instances and with certain procedures it has been found not necessary to use a mineral acid. It has also been found that in some instances and under certain conditions an alkaline selectivity- 50 modifying agent is of assistance when used with a frothing agent in the preferential

flotation-separation of certain sulfids from other sulfids, but so far as we are aware a froth flotation-separation has not been effected by the use in solution of an alkaline substance without the addition of a mineral-frothing agent, and the function of maintained alkalinity in the ore pulp has been to assist a frothing agent in froth flotation.

We have discovered that if the agitation 60 froth process be carried on in an ore pulp containing in solution an alkaline substance, such as carbonate of soda, and without the addition of any frothing agent other than the said alkaline substance, a froth of the 65 metalliferous mineral will rise to the surface and may be floated off or otherwise and separated from the gangue which remains in the pulp. This separation is preferably effected at a temperature in the neighborhood 70 of 130° Fahr.

The following is an example of our new process: Two lbs. of Broken Hill slimes were mixed with 7 lbs. water at 130° F., and soda ash equal to 22.4 lbs. per ton of the 75 slimes. The mixture was then thoroughly aerated by being agitated, with the result that a mixed concentrate assaying 29.5% lead, 35.2% zinc, 25.0 ozs. per ton silver was produced, giving recoveries of 90.0% lead, 80 92.7% zinc, and 91.5% silver.

If desired the resultant products may be retreated with or without the addition of fresh quantities of the alkaline substance, or by any other process, such as, for example, with the addition of oily organic or other frothing agents.

The concentrates obtained by this invention from ores containing mixed metalliferous minerals are found to be in a most suitable condition for preferential flotation-separation of one of the metalliferous minerals from other or others of the metalliferous minerals. The alkaline substances most suitable for addition to the ore pulp are the 90 carbonates of the alkaline metals, but other alkalis may be used. We prefer in most cases a crude sodium carbonate or soda ash.

In the application of this invention with various ores and under various conditions, 100 the example of the process above described may be modified without departing from

this invention, the conditions best adapted for any particular ore being determinable by tests as well known in this art.

We claim:

5. 1. A process of concentrating ores which consists in agitating and aerating an ore pulp containing in solution an alkaline substance, but without the addition of a frothing agent other than the said alkaline substance, so as to obtain a froth of concentrates, and separating the froth.
10. 2. A process of concentrating ores which consists in agitating and aerating an ore pulp containing in solution a salt of a mineral acid having an alkaline reaction, but without the addition of a frothing agent other than said salt, so as to obtain a froth of concentrates, and separating the froth.
15. 3. A process of concentrating ores which consists in agitating and aerating an ore pulp containing sodium carbonate in solution, but without the addition of a frothing agent other than said sodium carbonate, so as to obtain a froth of concentrates, and
20. separating the froth.
25. 4. A process of concentrating ores which consists in agitating and aerating a heated ore pulp containing in solution an alkaline substance, but without the addition of a frothing agent other than the said alkaline substance, so as to obtain a froth of concentrates, and separating the froth.

5. A process of concentrating ores which consists in agitating and aerating a heated ore pulp containing in solution a salt of a mineral acid having an alkaline reaction, but without the addition of a frothing agent other than said salt, so as to obtain a froth of concentrates, and separating the froth.

6. A process of concentrating ores which consists in agitating and aerating a heated ore pulp containing sodium carbonate in solution, but without the addition of a frothing agent other than said sodium carbonate, so as to obtain a froth of concentrates, and separating the froth.

In testimony whereof we, HENRY LAVERS and HENRY HOWARD GREENWAY, have affixed our signatures in presence of two subscribing witnesses.

HENRY LAVERS.

HENRY HOWARD GREENWAY.

Witnesses:

Wm. A. HACK,  
J. R. CULLEN.

In testimony whereof I, ALFRED HENRY PIPER LOWRY, have affixed my signature in presence of two subscribing witnesses.

ALFRED HENRY PIPER LOWRY.

Witnesses:

ARTHUR GORE COLLISON,  
FLORENCE MANTHORPE.